# EUROPEAN PATENT APPLICATION

(11) **EP 2 175 059 A1**
(43) Date of publication of application: **14.04.2010**
(21) Application number: 08460039.4
(22) Date of filing: 07.10.2008
(51) Int. Cl.: D04H 1/00, D01G 13/00

(54) **Wool yam**

(71) Applicant: Fabryka Dywanow Agnella S.A., 15-113 Bialystok (PL)
(72) Inventor: Jan Sobon, Jacek, 61 606 Poznan (PL); Rosinska, Krystyna, 15 794 Bialystok (PL); Dabrowska, Emilia, 16 010 Wasilkow (PL); Dmitruk, Helena, 15 661 Bialystok (PL)

(57) **Abstract**

The finished yam is made only of naturally coloured wool fibres already currently present in nature and originating from around the world ( British, Norwegian, European, South American and New Zealand wools are types commonly used). The finished yam is manufactured without any dyeing of the raw material. The yam composition is 100% naturally coloured wool. Special processing with impregnation agents is used to help protect natural colours against fading under the influence of UV radiation. The colours of the finished yam are achieved by blending up to 20% Crossbred, Swaledale, Blackface, Halfbred wool fibres, with up to 40% depigmented wool fibres, with up to 20% New Zealand wool fibres and up to 20% wool fibres of American, Libyan and European origin.

## Description

The present invention relates to wool yarn.

Generally, yarns are made using white virgin wool. They can then be coloured to shade using a dyeing process.

The nature of the invention is that the finished wool yarn is made using only naturally coloured fibres carefully selected for there natural pigment. The wool fibres chosen are already present in nature and originating from countries throughout the world such as; British, Norwegian, European, South/American and New Zealand wools. The finished yarn is manufactured without any dyeing of the raw material.

The yarn composition is from 100% natural coloured wool fibres. Special processing with impregnation agents protects these natural colours against fading under the influence of ultra violet (UV) radiation. The colour of the finished yarn is achieved by careful selection, blending, combinations of up to 20% Crossbred, Swaledale, Blackface, Halfbred wool fibres, with up to 40% depigmented wool fibres, up to 20% New Zealand wool fibres and up to 20% wool fibres of American, Libyan and European origin.

Using only naturally coloured yarn without the need for any dyeing process helps protect the natural environment because no effluent is created the same as during traditional dyeing.

Each individual colour of yarn is achieved by blending different quantities of British wools with European, New Zealand wools and other wool fibres from around the world depending on the shade required.

For example, cream beige, dark beige colours are produced by blending up to 50% depigmented wool fibres with up to 20% Crossbred wool fibres and up to 30% New Zealand wools.

Gray colours are obtained blending combinations of up to 50% Crossbred, Swaledale, Halfbred wool fibres with up to 20% Crossbred wool fibres and up to 30% New Zealand wool fibres.

Dark colours : brown, graphite are obtained by blending up to 40% depigmented wool fibres with up to 20% Crossbred wool fibres, with up to 20% European wool fibres and up to 20% South-American wool fibres.

## Claims

1. The finished wool yarn has a natural pigmentation, it is made by using only natural coloured fibres of wool which currently exist in nature, originating from all over the world. ( Types such as British, Norwegian, European, South/American and New Zealand wools are used), The finished yarn is manufactured without any dyeing process, with attractive colours achieved by exclusive selection, blending and carding. The finished yarn consists only of 100% wool fibres, specially processed with impregnation agents thus helping protect against fading under the influence of UV radiation.

2. Wool defined in claim 1, wherein the colours are obtained as a result of blending: combinations of up to 20% Crossbred , Swaledale, Blackface, Halfbred wool fibres with up to 40% depigmented wool fibres and up to 20% New Zealand wool fibres and up to 20% wool fibres of other origin: American, Libyan and European.
